

## UNITED STATES PATENT OFFICE

DAVID GESTETNER, OF TOTTENHAM HALE, LONDON, ENGLAND, ASSIGNOR TO D. GESTETNER, LIMITED, OF LONDON, ENGLAND

MANUFACTURE OF ROLLERS AND PARTICULARLY ROLLERS ADAPTED FOR USE AS PRINTING ROLLERS

No Drawing. Application filed May 31, 1927, Serial No. 195,604, and in Great Britain June 3, 1926.

This invention relates to the manufacture of rollers and particularly such as are adapted for use in the distribution of ink in printing and like operations and in the production of sheets or slabs or the like adapted for use in printing, lithography and in the offset process.

It is well known that gelatine compositions are commonly employed in the formation of printers' rollers, that is to say, the rollers employed in connection with printing machines for inking the faces of the type or other impression-producing means.

It would seem that the surface of gelatine compositions possesses certain desirable properties in this connection.

Hitherto, in the production of such rollers, the general practice has been to cast a body of a gelatine composition about a metal or wooden mandrel. In the course of use the surface of the gelatine composition becomes injured and it is necessary to recast the roller, that is to say to remove the gelatine composition from the mandrel and to form thereon a further body of a like composition. This operation necessitates a certain amount of skill and only in relatively few cases is the operation performed in the printing works.

Moreover, such gelatine compositions are sensitive to variation in temperature, that is to say a composition which is sufficiently elastic or resilient at a given temperature becomes too hard at a certain lower temperature and too soft or even fluid at a higher temperature. They are in fact gelatine compositions which are fluid at elevated temperatures but which at the normal temperature of the air exist as resilient or elastic masses.

It has been proposed to employ other materials in forming printing rollers, for instance sulphurized oil compositions, and, further, it has been proposed to provide rollers formed from resilient materials other than gelatine compositions, for instance sulphurized oils, with a coating of a gelatine composition which is similar to that at present used in forming printers' rollers and which is as above stated temperature sensitive.

Sulphurized oil compositions in many cases exhibit a certain degree of mechanical weakness which is perhaps best described as "shortness".

Thus, bodies of these compositions when subjected to certain stresses of no great magnitude rupture, displaying a conchoidal fracture.

Such rollers are therefore liable to be injured by the type faces when they are used for inking type.

One of the observations on which the present invention is based is that by the provision on the surfaces of bodies of compositions, possessing the before-mentioned properties or character of vulcanized oil compositions, of an attenuated coating of a flexible insolubilized gelatine composition, the resistance thereof to the destructive agencies to which they are subjected when used as inking rollers can be considerably increased.

The expression "attenuated coating" as used herein denotes generally coatings having a thickness of one-fortieth to one-fifteenth or one-tenth of a millimetre or even more so long as the coating does not by reason of its thickness exhibit a tendency to strip from the body of the roller.

According to the present invention dispersions of gelatine possessing both low viscosity and high concentration are employed.

Thus, dispersions of gelatine containing bodies which depress the gelating point of the dispersions may be used in forming the coating.

Preferably, the bodies, adapted to depress the gelating point, which may be present in the dispersions used are such that they may be removed or changed in character after the dispersion is applied to the body to be coated.

Usually the dispersions used are of such character that they are fluid at substantially the normal temperature of the air or at but slightly elevated temperatures.

Thus, in accordance with the invention, gelatine compositions, the hardening or setting of which is to be attributed to the evap-

oration of the whole or a portion of their content of solvent, may be used.

Alternatively, gelatine compositions, the setting point of which can be raised by treatment with suitable reagents, may be employed.

In a further alternative, dispersions of gelatine are employed in a sufficiently heated state to diminish their viscosity to a degree such that they may be applied to the roller and form thereon an attenuated coating or thin film.

Generally it is found preferable to use high grade gelatines in forming the compositions but in some cases glues of suitable qualities may be used.

In some cases liquid glues will be found suitable.

Preferably the gelatine coating is hardened by means of formaldehyde or by chromium compounds, the former being used for this purpose in the form of a solution or as vapour.

After the gelatine coating has set and after it has been hardened or coagulated the coating is treated to increase its flexibility, as for instance by impregnating it with glycerine or an equivalent material employed in the form of an aqueous solution.

During the time the roller is in use the proportion of glycerine in the coating may become reduced and the coating thus tends to develop brittleness; the original elasticity may in such case be restored by impregnating the coating with glycerine.

A further feature of the invention is concerned with the production of a roller provided with an attenuated coating of a gelatine composition which has a roughened, toothed or grained surface.

Thus in accordance with this feature of the invention a dispersion of gelatine may be sprayed on to the roller either before or after it has been provided with an attenuated coating of a gelatine composition.

Rollers having a roughened surface are particularly suitable for use in connection with offset printing machines and the graining of the surface of the roller may correspond with the graining of the surface of the member of the offset machine from which the offset impression is transferred.

The following is an example of a suitable composition for use in accordance with the invention:—

20 to 30 parts by weight of gelatine dispersed in 100 parts by weight of a mixture consisting of equal parts by volume of glacial acetic acid and water.

In carrying the invention into effect the gelatine composition may be applied to the body of the roller by a flowing, spraying or immersion operation.

Where a sufficiently thick but still attenuated coating cannot be obtained by a single

treatment of a roller with a gelatine composition the treatment may be repeated until a coating of the desired thickness is formed thereon.

While the invention is mainly concerned with rollers adapted for use as printers' rollers it is not confined to rollers for use for any particular purpose; for instance, the invention extends to rollers adapted for use as pressure rollers in connection with duplicating machines and to rollers for use in connection with offset printing machines adapted to perform the function of the so-called "blanket" provided in such machines.

Having now described my invention, what I claim as new and desire to secure by Letters Patent is:—

The process of producing rollers, sheets, slabs and the like which comprises immersing a suitably formed body of a vulcanized oil composition in a dispersion of gelatine which is fluid at temperatures slightly above normal temperature of the air, allowing the excess of gelatine to drain from said body, subjecting the gelatine to the action of an insolubilizing agent and immersing the same in a hygroscopic softening agent.

In testimony whereof I have signed my name to this specification.

DAVID GESTETNER.

95

100

105

110

115

120

125

130